

# UNITED STATES PATENT OFFICE.

ADOLF SWOBODA, OF VIENNA, AUSTRIA-HUNGARY, ASSIGNOR OF  
ONE-HALF TO WALTER BOKMAYER, OF MODLING, NEAR  
VIENNA, AUSTRIA-HUNGARY.

## MATCH.

No. 810,363.

Specification of Letters Patent.

Patented Jan. 16, 1906.

Application filed July 12, 1905. Serial No. 269,422.

*To all whom it may concern:*

Be it known that I, ADOLF SWOBODA, a subject of the Emperor of Austria-Hungary, residing at Vienna, Austria-Hungary, have invented a certain new and useful Improvement in Matches, of which the following is a specification.

This invention relates to a composition used for the manufacture of improved igniting compounds for matches of all kinds, (wax matches and others,) these compounds distinguishing from other compounds of similar kind in as far as the same are free from poisonous phosphorus and sulfur and containing besides other known igniting materials a certain amount of substances that give to the compounds qualities hitherto unknown.

The heads of all matches now in use the ignition of which is required to take place upon any rubbing-surface whatever contain the constituent parts necessary for ignition, viz: chlorate of potassium, amorphous phosphorus, and sulfur, in a mixture to which are added, according to prescriptions, some other substances serving principally as filling or binding materials. Experience has shown that all these igniting compounds do not turn out well in practice, because they are subject to the same defects, and the danger of exploding during manufacture of such igniting compounds has not yet been entirely prevented.

Now I have found that when adding a mixture consisting of three parts, of weight, of finely-powdered cork, fifteen parts, of weight, of iron minium, twenty-three parts, of weight, of flour, the whole intimately mixed with forty parts, of weight, of water to igniting compounds already known, the constituent parts and proportions of which are indicated in the following example, an igniting compound free of poisonous phosphorus and sulfur may be obtained in the cold without any danger and without development of injurious vapors. The resulting compound allows the manufacture of matches of all kinds (of paraffined or sulfured wood splits or of wax sticks) that are ignited when rubbed upon any rubbing-surface whatever.

The original compound used for making the improved igniting compound consists of about fifty-seven parts, of weight, of chlorate of potassium, about seven parts, of weight, of

red chromate potassium, ( $K_2CrO_4$ ), about seven parts, of weight, of amorphous phosphorus, about fifteen parts, of weight, of powdered glass, and about thirty parts, of weight, of gum-arabic dissolved in about forty parts, of weight, of water.

By means of the composition before specified an improved igniting compound may be manufactured in the cold, preferably in the following manner: Thirty parts, of weight, of gum-arabic are dissolved in forty parts, of weight, of water. To this solution are added fifty-seven parts, of weight, of finely-powdered chlorate of potassium. After suspension of the chlorate of potassium seven parts, of weight, of chromate of potassium, seven parts, of weight, of amorphous phosphorus, and fifteen parts, of weight, of powdered glass are poured into this solution, and the whole is intimately mixed by stirring. A paste is then prepared of three parts, of weight, of powdered cork, fifteen parts, of weight, of iron minium, and twenty-three parts, of weight, of flour, the whole mixed with forty parts, of weight, of water. This paste is added to the liquid mixture before described, and the whole mass is again intimately mixed.

The improved igniting compound permits of manufacturing of matches without a preceding drying, preheating, or paraffining of the splints, and besides this it offers the following very important advantages: Ignition of the carrier of the igniting compound—as, for example, splints or wax sticks—is perfectly assured, and every danger of exploding during preparation of the igniting compound is removed. An excessive hardening of the heads of the matches is not to be feared, and development of oxygen by the chlorate of potassium during ignition of the match is facilitated to such an extent that no sulfur is required for ignition of the wood. The effect of the several constituent parts of the paste—viz., of the cork, iron minium, and flour—is the following: The powdered cork does not only prevent depositing of the constituents of the igniting compound, but, contrary to powdered wood, it prevents a sudden flaring up of the igniting compound and makes the latter soft and supple. The flour makes the compound consistent to such an extent as required for the dipping process. The iron

minium causes the heads of matches to assume a rounded shape at top, while without the addition of iron minium the heads would have prolonged thread-like ends.

5. The finished head of the matches may be covered with a layer of grease, protecting same against all atmospheric influences and preventing self-ignition during manufacture or transport.

10. What I claim, and desire to secure by Letters Patent, is—

1. The composition of matter consisting of powdered cork, iron minium, flour and water substantially as described and for the purpose specified.

2. The herein-described composition of matter as additional matter to igniting compounds for matches of all kinds consisting of three parts of weight of powdered cork, fifteen parts of weight of iron minium, twenty-

three parts of weight of flour and forty parts of weight of water, substantially as described.

3. The herein-described composition of matter consisting of powdered cork, iron minium, flour and water in combination with an igniting compound for matches consisting of: fifty-seven parts of weight of chlorate of potassium, seven parts of weight of red chromate of potassium, seven parts of weight of amorphous phosphorus, fifteen parts of weight of powdered glass, thirty parts of weight of gum-arabic and forty parts of weight of water, substantially as described.

In testimony whereof I affix my signature in presence of two witnesses.

ADOLF SWOBODA.

Witnesses:

SIEGERIED NEUTER,  
ALVESTO S. HOGUE.